

I. L. ROBERTS.

MANUFACTURE OF WATERPROOF ARTICLES FROM FIBROUS MATERIALS.

APPLICATION FILED MAY 26, 1908.

921,001.

Patented May 11, 1909.



Witnesses:

Raphael Letter  
S.S. Dunham.

I. L. Roberts,  
Inventor

By his Attorneys  
Messrs. Page & Cooper

# UNITED STATES PATENT OFFICE.

ISAIAH L. ROBERTS, OF LOCKPORT, NEW YORK.

## MANUFACTURE OF WATERPROOF ARTICLES FROM FIBROUS MATERIALS.

No. 921,001.

Specification of Letters Patent.

Patented May 11, 1909.

Application filed May 26, 1908. Serial No. 435,130.

To all whom it may concern:

Be it known that I, ISAIAH L. ROBERTS, a citizen of the United States, residing at Lockport, in the county of Niagara and State of New York, have invented certain new and useful Improvements in the Manufacture of Waterproof Articles from Fibrous Materials, of which the following is a specification.

10 My invention relates to the manufacture of waterproof articles, for example tubes, rods, vessels, plates, sheets, etc., composed of fibrous material such as wood pulp, strawboard, paper, cotton and other cellulose products, and has for its chief object to provide a simple, cheap, and withal thoroughly effective process for rendering such articles non-absorptive or "waterproof."

Heretofore it has been customary to impregnate the articles, or fill the pores thereof, with waterproofing material, or to coat the surface of the article with suitable impervious material, or to treat the article in the wet way with various chemical agents.

25 However successful for the purpose the prior methods may have proved, all those with which I am familiar, particularly the methods just referred to, possess certain drawbacks. Chief among these drawbacks are 30 the matter of expense and, in some of the processes at least, the fact that the weight of the article is largely increased by the considerable quantity of impregnating or coating material employed. Furthermore, such

35 articles when coated or impregnated have little or none of their natural resiliency and as a result are liable to breakage under strains that otherwise might cause merely a temporary distortion. I have therefore

40 been led to devise my present invention, by which I am able to produce fibrous articles which are thoroughly waterproof at low cost, and at the same time of lighter weight, stronger texture and less liability to break, 45 without increasing the weight thereof or the liability of breakage.

The most important feature of my invention resides in the discovery that on heating an article composed of fibrous cellulose the 50 fibers of which have some water repellent substance or substances, such as oil or paraffin, well distributed on and among them or naturally in them, in minute or attenuated quantities so minute in fact, as not to be palpable to the touch or visible to the eye, the article will repel water completely, acting in

this respect a good deal like the feathers of birds. The treatment with the water-repellent substance can be effected in various ways and with various materials, but the organic oils appear to give the best results. For example, in making waterproof cotton cloth, the oil may be blown or "atomized" on to the dry cotton fibers before spinning. Or, if wax is used, the same may be pulverized or 65 melted and then blown in a fine spray on to the cotton. In the case of wood-pulp, strawboard, etc., the oil or powdered wax may be put into the pulping machines and thoroughly mixed with the fibers. This method 70 applies both to original pulping or to the repulping of pulp-board, strawboard, etc. In the case of articles made wholly or in part of repulped printed paper, I have found the oil of the printers' ink is usually sufficient for the 75 purpose desired; but if not, additional water-repellent oil or wax may be used. From the material treated as above or in an equivalent manner, the cloth, vessels, or other articles or products are made by the usual methods, 80 and are then heated. The heating is preferably effected in a closed or partially closed chamber or oven, and is carried to a temperature above that of boiling water to a point sufficient to cause the oil or wax to be 85 thoroughly incorporated with the fibers. The temperature required for the purpose depends upon the nature of the material and the article, but in no case have I found it necessary to go above 400° F., and in many 90 cases a temperature as low as 240° F. has been found sufficient. The length of time during which the heating should be maintained also varies, but in general two to 95 eighteen hours will be found sufficient. At the lower temperature it is necessary to heat the article longer than at the higher temperature, and similarly thick-walled articles need longer heating at any given temperature than those whose walls are thinner. In order to 100 be sure of the results, the heating must be carried on for a period and at a temperature sufficient to partially decompose the fibers of the article and to effect a combination of the oils, gums or waxes therewith. At temperatures between the boiling point of water and about 400° F. the heating has the effect of strengthening the articles, but at higher temperatures they are weakened.

105 While the use of oil or other water-repellent substance is believed to be necessary for the best results, I have found that simple

heating of articles made of wood-pulp, rag-pulp, etc., will give them water repellent qualities to a marked degree,—sufficient, at least, to serve many purposes where substantially waterproof articles are desired, as for example receptacles for the storage or shipment of merchandise. Such articles, made of material of the kind referred to and heated to a temperature of from 240° to 400° F. for 10 from two to eighteen hours or longer, (the higher the temperature the shorter the time, and vice versa), will maintain their contents dry for a long time even under adverse conditions of the atmosphere or weather. Straw-board, however, does not do so well with simple heating, but should have the treatment with water-repellent oil or wax, as herein described.

If water vapor is added to the atmosphere 20 in the oven in which the articles are heated it will in some cases improve the results. For this purpose an open vessel containing a small quantity of water may be placed in the oven, or steam may be injected into the oven. 25 The use of water vapor in the atmosphere of the oven does not result in making the articles moist or damp since the temperature is above the condensing point of water.

A convenient type of heating apparatus 30 for use in practicing my invention is illustrated in the annexed drawing. The figure there given shows the heating oven in vertical section.

The oven A, having heat-insulating walls, 35 contains a coiled heating pipe B, provided with suitable valves C, D, for controlling the flow of the steam or other heating medium therethrough. Close above the heating coil, which is located at the bottom of the oven, 40 are two perforated iron plates, E, F. On the lower plate may be placed a vessel H, containing water. On the upper plate are placed the articles to be treated, which are preferably disposed so as to permit the atmosphere 45 of the oven to readily reach all parts. The articles are introduced through an opening in the side of the oven, which is then closed tightly by a closure or door I.

The oven being charged, the steam or other 50 heating medium is let into the heating coil.

The water in the vessel H soon begins to vaporize, and the steam therefrom displaces the air, which is allowed to escape through a cock J, conveniently located. When the desired temperature has been reached, as can 55 be determined from a thermometer, as K, extending into the oven at any convenient point, the heat is maintained at about that degree for the time desired, after which the articles are removed and allowed to cool. Of course in the case of treatment without water the vessel H is omitted or merely left empty, as desired.

It is to be understood that the apparatus herein shown is not an essential part of my 65 invention, which being a process, is not confined to any particular type or kind of apparatus for practicing it.

What I claim is:

1. The herein described method of manufacturing waterproof articles, which consists in forming an article of pulped cellulose or woody material, and heating the article to a temperature sufficiently high and for a time sufficiently long, as described, to render the 75 article substantially waterproof.

2. The herein described method of manufacturing waterproof articles, which consists in forming an article of pulped cellulose or woody fibers treated with a water-repelling 80 substance, and heating the article for a sufficient time and at a temperature sufficiently high, as described, to render the article waterproof.

3. The herein described method of manufacturing waterproof articles, which consists in forming an article of pulped cellulose or woody material, and heating the article to a temperature above the boiling point of water for approximately two hours or longer. 85 90

4. The herein described method of manufacturing waterproof articles, which consists in forming an article of pulped cellulose or woody material, and heating the article to a temperature of from 240° to 400° F. for approximately two hours or longer. 95

ISAIAH L. ROBERTS.

Witnesses:

M. LAWSON DYER,  
S. S. DUNHAM.